

## UNITED STATES PATENT OFFICE

2,072,670

## REDUCING DUSTING IN THE MANUFACTURE OF COATED PAPER

Louis C. Fleck, Appleton, Wis., assignor, by mesne assignments, to K. C. M. Company, Dayton, Ohio, a corporation of Delaware

No Drawing. Application June 29, 1934,  
Serial No. 732,994

10 Claims. (Cl. 92—40)

In the operation of coating paper with materials having a mineral constituent considerable trouble has been experienced from a phenomenon known in mill parlance as "dusting". This is due 5 mainly to the fact that the mineral coating matter is insufficiently bonded together and to the paper, and results in much of the coating coming off as a dust cloud (in aggravated cases) at the rewinder, or sticking to the calender rolls until 10 it has built up scales, which eventually detach themselves from the roll and go along with the paper; or it shows up in the print shop where it builds up on the tympan or backing sheet or sheets for the sheet of paper on which the printing is being done.

This "dusting" phenomenon manifests itself mainly in what are known as continuous processes; that is, processes wherein the coating is applied by coating rolls, dipping, or otherwise to 20 the partly dried paper web as it comes from the web forming machine, an example of this process being shown in Letters Patent to Germanson and Kranhold, No. 1,918,095, granted July 11, 1933.

I have discovered that dusting may be greatly 25 reduced, and in many cases practically eliminated, by keeping the viscosity of the coating liquid substantially constant or uniform, and this is preferably done by suitably controlling the temperature of the coating fluid.

30 In processes such as I have described the partly dried paper web coming to the coating press is hot by reason of heat absorbed from the drying rolls, and the result is that the coating material through or in contact with which the hot web 35 passes at the coating press, itself becomes hot.

As to the reasons why hot coating causes dusting, it is believed to be largely due to the reduced viscosity of the liquid portion of the coating at the higher temperature, which in the case of such 40 coating mixtures as casein, clay and water, permits the liquid portion to penetrate the paper web to a greater extent, carrying with it the dissolved casein, and leaving the mineral matter (clay) on the surface without sufficient binder 45 to hold it together and in place. Furthermore, if the coating is held for some time at an elevated temperature it undergoes some chemical and even bacterial decomposition, which is also believed to deleteriously affect its binding power.

50 The reduction in temperature of the coating fluid may be effected either by cooling the hot web before it encounters the coating mixture, as, for example by passing it over one or more cooling cylinders through which a cooling medium 55 (such as brine) is circulated, or by cooling the

coating mixture itself as, for example, water-jacketing the mixture pan and the pipe lines through which the mixture circulates and placing cooling coils in the coating storage tanks, or both. Since mechanical embodiments of these 5 suggested cooling methods are obvious, illustrations thereof in the form of drawings are believed to be unnecessary.

The dusting nuisance above described is harmful in at least two ways. In the first place it impairs 10 the quality of the coated product, and in the second place, it fouls the atmosphere of the mill room in which the machine attendants are employed.

It has been observed in laboratory studies that 15 sheets of paper dipped or treated with hot aqueous coating solutions and pressed between rolls tend to disintegrate, loosen, swell and roughen the surface constituents of the sheet more than sheets of paper dipped or treated with a cold 20 aqueous coating mixture. This roughening effect and loosening of the bonds of the fibers to one another results in a finished sheet which has fibers standing up on the surface. Drying the 25 swelled fibers also results in shrinkage and distortion of coating on the fibers. When such a sheet is calendered or brushed, coating and distended fibers rupture and break off on and under the surfaces of the paper. This results in what 30 is commonly known as dust.

The application of a cold aqueous coating mixture no doubt prevents excessive accelerated 35 swelling, decreases the tendency of breaking the bonds between fibers and results in a comparatively smooth, compact sheet. The smoother and more compact the sheet, the less danger there is of fibers and coating breaking off on calendering to form the so-called dust.

I have found by experiments that the above 40 described method of abating or lessening this dusting nuisance is most effective in the case of coatings which contain casein as the binder, and somewhat less so in the case of starch coatings. Undoubtedly it may also be used to advantage 45 with coating mixtures containing binders other than casein and starch.

I claim:

1. The process of preparing a substantially 50 non—"dusting" paper, as part of a continuous paper making operation, which comprises applying to a heated, partially dried web a coating composition containing an adhesive liquid fraction and an insoluble solid fraction, the coating composition at the point of application being maintained at a temperature sufficiently low, and 55

- at a viscosity sufficiently high, to prevent separation of the liquid fraction from the solid fraction during the coating operation.
2. The process as defined in claim 1 in which the said temperature and viscosity are maintained by continuously abstracting from the coating mixture the heat imparted thereto by the heated web.
3. The process as defined in claim 1 wherein the said temperature and viscosity are maintained by continuously abstracting from the coating mixture substantially at its point of application to the web the heat imparted to the coating mixture by the heated web.
4. The process as defined in claim 1 in which the said temperature and viscosity are maintained by continuously subjecting the coating mixture to the influence of a cooling medium to abstract therefrom the heat imparted thereto by the heated web.
5. The process as defined in claim 1 in which the said temperature and viscosity are maintained by continuously subjecting the heated web to the influence of a cooling medium prior to its contact with the coating mixture.
6. In a process of preparing a substantially non-“dusting” paper, as part of a continuous paper making operation, wherein the wet web is heated immediately before receiving a coating composition, containing an adhesive liquid fraction and an insoluble solid fraction, to partially dry the same, the improvement of preventing the thus heated web from causing such rapid penetration by the adhesive liquid fraction as to cause separation from the latter of the solid fraction, resulting in “dusting”, such improvement comprising the maintenance of the temperature and viscosity of the mixture, at the point of application to the web, sufficiently low and high respectively to prevent such undesirable, rapid penetration.
7. The process as defined in claim 6 in which the said temperature and viscosity are maintained by continuously abstracting from the coating mixture the heat imparted thereto by the heated web.
8. The process as defined in claim 6 wherein the said temperature and viscosity are maintained by continuously abstracting from the coating mixture substantially at its point of application to the web the heat imparted to the coating mixture by the heated web.
9. The process as defined in claim 6 in which the said temperature and viscosity are maintained by continuously subjecting the coating mixture to the influence of a cooling medium to abstract therefrom the heat imparted thereto by the heated web.
10. The process as defined in claim 6 in which the said temperature and viscosity are maintained by continuously subjecting the heated web to the influence of a cooling medium prior to its contact with the coating mixture.

LOUIS C. FLECK.